# EUROPEAN PATENT SPECIFICATION

(11) **EP 0 547 127 B1**
(45) Date of publication and mention of the grant of the patent: **24.09.1997**
(21) Application number: 91916342.8
(22) Date of filing: 06.08.1991
(51) Int. Cl.: C10M 169/04, C10M 107/34, C10N 40/08

(54) **Process for imparting fire resistance to a hydraulic system**
Verfahren zur Verbesserung der Feuerbeständigkeit von Hydrauliksysteme.
Procédé pour d'amélioration de la résistance au feu d'un système hydraulique

(30) Priority: 31.08.1990 US 576301
(43) Date of publication of application: 23.06.1993
(73) Proprietor: OLIN CORPORATION, Cheshire, CT 06410-0586 (US)
(72) Inventor: MILLER, Philip, R., Hamden, CT 06517 (US)
(74) Representative: Baker, Colin John
(86) International application number: US9105573
(87) International publication number: WO9204428

(56) References cited:
- US-A- 2 499 723
- US-A- 3 567 639
- US-A- 3 981 850
- European Patent Application (LEVRERO et al.) 21 March 1990 (Note page 3, lines 11-50).

## Description

This invention relates generally to hydraulic fluid compositions and, more specifically, to hydraulic fluids characterized by enhanced fire resistance.

In the past, polyalkylene glycol-based hydraulic fluids have generally required the presence of water therein in order to provide a degree of fire resistance sufficient to meet the Factory Mutual Research, Group I, Class No. 6930 approval (so-called "FM approval") with regard to the flame resistance of the fluid. Water is undesirable as an additive in hydraulic fluids for several reasons, most notably due to operating pressure limitations imparted by the vapor pressure of water and corrosion problems caused by water on the metal surfaces of the hydraulic system.

In view of the above, non-aqueous hydraulic fluids that exhibit an improved combination of flame retardancy and shear stability would be highly desired by the hydraulic fluid manufacturing community.

The present invention relates to a process for imparting flame retardancy, hydrolytic stability, and reduced wear characteristics to a hydraulic system which comprises adding to the hydraulic system a hydraulic fluid composition comprising:
(a) a polyalkylene glycol base fluid, and
(b) as an anti-mist additive, an alkylene-vinyl ester copolymer having a molecular weight of between 5,000 and 100,000 and soluble in said base fluid.

These and other aspects will become apparent upon reading the following detailed description of the invention.

In accordance with the present invention, it has now been surprisingly found that a hydraulic fluid composition can be provided that provides excellent anti-wear properties as well as enhanced flame retardancy over time during use. The hydraulic fluid is polyalkylene glycol based and contains an anti-mist additive exhibiting an improved shear-stable characteristic relative to those utilized in polyol ester type hydraulic fluids.

The polyalkylene glycols useful as the base fluid in the hydraulic fluids of the present invention are generally anionically or cationically catalyzed using, for example, an alkali metal salt of a lower alkanol initiator. An illustrative example is a potassium hydroxide catalyzed butanol initiated polypropylene glycol. The various polyalkylene glycols, including monols, diols, triols, and the like, are well-known in the art and are commercially available, for example, under various trademarks, including Olin Corporation's POLY-G trademark, Union Carbide Corporation's UCON trademark, and BASF Corporation's PLURACOL trademark.

The anti-mist additive useful in the present invention is an alkylene-vinyl ester copolymer having a molecular weight of between 5,000 and 100,000, wherein the alkylene compound is preferably selected from the group consisting of ethylene, propylene, butylene, and combinations thereof. The copolymer can be a random or block-type copolymer with the ratio of alkylene groups to vinyl ester groups in the copolymer being between 1:10 and 10:1 with the proviso that the copolymer be soluble in the base fluid. The most preferred copolymer is an ethylene-vinyl ester copolymer commercially available as V-152, a product of Functional Products Corporation of Cleveland, Ohio. The copolymer is suitably prepared using known techniques for ethylene-vinyl ester copolymerizations as disclosed, for example, in U.S. Patents 3,254,063 and 3,591,502.

Illustratively, the alkylene-vinyl ester copolymer is suitably prepared by copolymerizing the alkylene compound (e.g., ethylene, propylene, butylene, or combinations thereof) with a copolymerizable unsaturated ketone. Suitable ketones include, for example vinyl methyl ketone, vinyl n-octyl ketone, vinyl-isooctyl ketone, vinyl dodecyl ketone, vinyl-cyclohexyl ketone, 3-pentene-2-one, and combinations thereof. The molar percent of alkylene compound to ketone is suitably between 5 and 80 percent based upon the total amount of alkylene compound plus ketone employed to produce the copolymer.

The amount of anti-mist additive in the hydraulic fluid of the present invention is preferably between 0.1 and 20 weight percent, and more preferably between 0.5 and 10 weight percent based upon the total amount of anti-mist additive plus base fluid in the hydraulic fluid.

The hydraulic fluid of the present invention is non-aqueous or "essentially water free" which is intended to designate that the hydraulic fluid contains no more than 5 weight percent water, preferably no more than 2 weight percent water, based upon the weight of the hydraulic fluid.

In compositions of this invention, it is essential that both the component (a) and the component (b) be present in order to provide the desired flame retardancy and anti-wear properties. Additional optional additives are also suitably employed as desired, including, for example, the functional fluids of this invention will normally contain very minor amounts, typically from 0.01% to 5.0% by weight of various additives of the type commonly incorporated in formulating hydraulic fluids and lubricants such as rust and oxidation inhibitors, corrosion inhibitors, metal passivators, antiwear agents and other special purpose additives.

Rust and corrosion inhibitors and metal passivators suitably employed include tolyltriazole, benzothiazole and benzotriazole and their derivatives, alkyl and aryl phosphites and sarcosine and succinic acid derivatives. Antioxidants include dialkylthiodi proprionate, for example, dilaurylthiodiproprionate etc. organic amines, for example, dioctyldiphenylamine, phenylnaphthylamine, hindered phenols, phenothiazine, etc. Antiwear additives include dithiophosphates, amine phosphites, organo-molybdenum compounds, phosphorothionates, carbamates, etc. The suitably of such optional additives will depend upon the operating conditions, and the service requirements for the particular application that the hydraulic fluid is employed in. Except for the requirements given above, the relative proportions of and the maximum amount of each of these components and the combination thereof that should be present is not critical to the present invention. Economic factors also help determine what optimum amounts should be used. If used, the optional additives are suitably employed in an amount up to 40 weight percent base upon the total weight of the hydraulic fluid.

The hydraulic fluid composition of the present invention preferably has a viscosity of between 15 and 3000 centistokes at 40°C.

The following examples are intended to illustrate, but in no way limit the scope of, the present invention.

### Example 1

### Preparation of Hydraulic Fluids and Pump Testing Thereof

Hydraulic fluid compositions reflecting the present invention were prepared in accordance with the following procedure utilizing the following formulation:

| Component Amount | |
|---|---|
| Formulation Components | (parts by weight) |
| POLY-G WI-285 (a butanol-initiated polypropylene glycol) | 95.8 |
| Phenothiazine | 0.5 |
| V-152 (ethylene-vinyl ester copolymer) | 3.0 |
| Triphenylphosphorothionate | 0.5 |
| Ciba Geigy Corps IRGALUBE 349 | 0.2 |

A commercially available polyol ester hydraulic fluid was used as a comparison, namely Cosmolubric® HF130 hydraulic fluid manufactured by E.F. Houghton Co. of Valley Forge, PA.

The formulations were tested using a laboratory hydraulic fluid pump test in accordance with ASTM-D2882 in order to measure the extent of pump wear resulting from the use of a specific fluid. Briefly, this test is conducted as follows:

Five gallons of a hydraulic fluid are circulated through a rotary vane pump system for 100 hours at a pump speed of 1200±60 rpm and a pump outlet pressure of 1.41x10⁶±2.81x10⁴ kg/m² (2000±40 psi). Fluid temperature at the pump inlet is 65.6±2.8°C (150±5°F). The result obtained is the total cam ring and vane (12) weight losses during the test.

The results of several pump wear tests ranged from 0.1 mg to 10.0 mg, indicating that this fluid is a premium performance hydraulic fluid. In comparison, the polyol ester hydraulic fluid wear amount ranged from 2.0 - 15 mg of weight loss during the 100 hour wear test.

The hydraulic fluids were also tested for fire resistance in accordance with the test procedure of Factory Mutual Research, Group II, Class No. 6930. Briefly, this test was conducted as follows:

A sample of fluid is heated to 60°C (140°F) in a steel container, then pressurized to 7.03x10⁵kg/m² (1000 psig) with nitrogen. The sample is discharged into an open space from a 80° hollow cone HAGO oil burner bozzle rated for 5.67 litres/hr (1.5 gal/hr) at 7.03x10⁴kg/m² (100 psig). This apparatus is used for both the flame propagation and hot surface tests described below:

Flame propagation test - A propane torch is introduced into an atomized spray for each fluid at points of 15.2 cm (6 inches) and 45.7 cm (18 inches) from the nozzle tip.

Ten attempts at ignition are made at each distance and any resulting fluid ignition is timed. Ignition lasting more than 5 seconds for any one of the ten attempts is considered a failure.

Hot Surface Ignition Test - A steel channel iron inclined 30° from the horizontal and equipped with side heat shields is heated from below by two propane-air burners to 704°C (1300°F). The burners are turned off, then fluid is discharged for 60 seconds at a distance of 15.2 cm (6 inches) The fluid can pass if ignition occurs, but the flame must not follow the spray when directed away from the hot surface.

The results of the fire resistance testing indicated that the polyalkylene glycol-containing compositions of the present invention passed the test and maintained their fire resistance for a time period of at least three times longer than the comparison polyol-ester type fluid (24 hours on average versus less than 8 hours on average for the comparison fluid in the pump test). This is based on periodic sampling of the two fluids during ASTM D2882 pump testing. It must be noted that the equipment used as part of this pump stand includes a pressure control valve thus creating an extreme shear condition, the degree of which is not experienced in normal field service. It is also noted that this fire resistance test was also performed on an analogous formulation to that described above, but replacing the butanol-initiated polypropylene glycol with a polypropylene glycol diol. This analogous formulation also passed the fire resistance test.

The fluids were also analyzed by GPC in order to determine the loss in molecular weight of the anti-mist additive utilized in the present invention as compared to the additive utilized in the comparison fluid. The additive of the present invention did decrease in molecular weight with time in the pump but did not change significantly in concentration in the hydraulic fluid formulation over time. In contrast, the comparison fluid suffered a decrease both in molecular weight and in concentration in the comparison hydraulic fluid over time in the pump during the period of the pump test.

## Claims

1. A process for imparting flame retardancy and reduced wear characteristics to a hydraulic system which comprises adding to the hydraulic system a hydraulic fluid composition comprising:
(a) a polyalkylene glycol base fluid, and
(b) as an anti-mist additive, an alkylene-vinyl ester copolymer having a molecular weight of between 5,000 and 100,000 and soluble in said base fluid, wherein the ratio of alkylene groups to vinyl ester groups in the copolymer is between 1:10 and 10:1, and wherein said anti-mist additive is present in an amount of between 0.1 and 20 weight percent based upon the total amount of anti-mist additive plus base fluid in the composition

2. The process of claim 1 characterized in that said polyalkylene glycol base fluid is selected from polyethylene glycol, polypropyleneglycol, polybutylene glycol, and combinations thereof.

3. The process of claim 1 or claim 2 characterized in that said alkylene-vinyl ester copolymer employs alkylene moieties selected from ethylene, propylene, butylene, and combinations thereof.

4. The process of claim 1 characterized in that said polyalkylene glycol base fluid is a lower alkanol-started polyalkylene glycol.

## Patentansprüche

1. Verfahren zur Verbesserung der Feuerbeständigkeit und Reduzierung der Verschleißeigenschaften eines hydraulischen Systems, wobei zu dem hydraulischen System eine Hydraulikfluidzusammensetzung gegeben wird, enthaltend:
(a) ein Fluid auf Polyalkylenglykolbasis und
(b) ein Alkylenvinylestercopolymer als Zusatzstoff gegen Nebelbildung, welches ein Molekulargewicht zwischen 5.000 und 100.000 besitzt und in dem Basisfluid löslich ist, wobei das Verhältnis der Alkylengruppen zu den Vinylestergruppen in dem Copolymeren zwischen 1:10 und 10:1 liegt, und wobei der Zusatzstoff gegen Nebelbildung in einer Menge zwischen 0,1 und 20 Gew.%, bezogen auf die Gesamtmenge des Zusatzstoffes gegen Nebelbildung und Basisfluid in der Zusammensetzunq, vorliegt.

2. Verfahren gemäß Anspruch 1, dadurch gekennzeichnet, daß es sich bei dem Fluid auf Polyalkylenglykolbasis um Polyethylenglykol, Polypropylenglykol, Polybutylenglykol und/oder deren Kombinationen handelt.

3. Verfahren gemäß Anspruch 1 oder 2, dadurch gekennzeichnet, daß das Alkylenvinylestercopolymer die Alkylenanteile Ethylen, Propylen, Butylen und/oder deren Kombinationen aufweist.

4. Verfahren gemäß Anspruch 1, dadurch gekennzeichnet, daß das Fluid auf Polyalkylenglykolbasis ein niederes, alkanolgestartetes Polyalkylenglykol ist

## Revendications

1. Procédé permettant de conférer des caractéristiques ignifuges et de résistance à l'usure à un système hydraulique, procédé qui consiste à ajouter dans le système hydraulique une composition de fluide hydraulique comprenant :
(a) un fluide de base de polyalkylène glycol, et
(b) un copolymère d'ester d'alkylène vinylique comme additif anti-buée de poids moléculaire compris entre 5.000 et 100.000 et soluble dans ledit fluide de base, dans lequel le rapport des groupes alkylènes aux groupes d'ester vinylique est compris entre 1:10 et 10:1, et dans lequel l'additif anti-buée est présent selon une quantité comprise entre 0,1 et 20 pour cent en poids sur la base de la quantité totale d'additif anti-buée plus le fluide de base dans la composition.

2. Procédé selon la revendication 1, caractérisé en ce que le fluide de base de polyalkylène glycol est choisi dans le groupe formé par le polyéthylène glycol, le polypropylène glycol, le polybutylène glycol et les mélanges de ceux-ci.

3. Procédé selon l'une quelconque des revendications 1 ou 2, caractérisé en ce que le copolymère d'ester d'alkylène vinylique utilise des fractions d'alkylène choisies dans le groupe formé par l'éthylène, le propylène, le butylène et les mélanges de ceux-ci.

4. Procédé selon la revendication 1, caractérisé en ce que le fluide de base de polyalkylène glycol est un polyalkylène glycol initié à partir d'alcanol inférieur.
